# EUROPEAN PATENT SPECIFICATION

(11) **EP 1 570 114 B1**
(45) Date of publication and mention of the grant of the patent: **19.04.2006**
(21) Application number: 03778571.4
(22) Date of filing: 02.12.2003
(51) Int. Cl.: C25C 3/00, C22B 3/00, C22B 34/14

(54) **SEPARATION OF METALS**
TRENNUNG VON METALLEN
SEPARATION DE METAUX

(30) Priority: 05.12.2002 GB 0228322
(43) Date of publication of application: 07.09.2005
(73) Proprietor: British Nuclear Fuels PLC, Warrington, Cheshire WA3 6AS (GB)
(72) Inventor: LEWIN, Robert, Glyn, c/o British Nuclear Fuels plc, Seascale, Cumbria CA20 1PG (GB); THIED, Robert, C., c/o British Nuclear Fuels Plc, Seascale, Cumbria CA20 1PG (GB)
(74) Representative: Harrison Goddard Foote
(86) International application number: PCT/GB2003/005238
(87) International publication number: WO 2004/050955

(56) References cited:
- WO-A-01/41152
- WO-A-99/64638
- WO-A-02/066712
- US-A- 4 762 694
- US-A- 4 923 577
- GOURISHANKAR KARTHICK ET AL: "Electrochemical reduction of metal oxides in molten salts" 2002, LIGHT MET (WARRENDALE PA); LIGHT METALS: PROCEEDINGS OF SESSIONS, TMS ANNUAL MEETING (WARRENDALE, PENNSYLVANIA) 2002, PAGE(S) 1075 - 1082 , XP009038370

## Description

### Field of the Invention

This invention relates to a method for the separation of metals from mixtures of metal oxides and relies on the selective reduction of certain oxides to the metals, whilst the other metals remain in the form of the oxides. The method of the present invention finds particular application in the separation of transition metals, lanthanides and actinides.

### Background to the Invention

The prior art teaches the use of molten salts in the separation of metals and metal oxides in molten salt media. As used herein, the term "molten salts" is intended to cover salts such as lithium chloride which melts at an elevated temperature and also ionic liquids which typically are liquid at room temperature or which melt at a temperature up to about 300°C. Such techniques have found particular application in the nuclear industry, where two well-established processes are available for the treatment of irradiated nuclear fuel.

The first of these processes, the Dimitrovgrad SSC-RIAR process, makes use of chemical oxidants (chlorine and oxygen gases) to react with powdered uranium dioxide fuel to form higher oxidation state compounds such as UO₂Cl₂ which are soluble in the molten salt. In an electrochemical cell the uranium compounds are reduced to UO₂ at the cathode, forming a solid deposit. This process has both technical and environmental limitations.

The second process, developed by the Argonne National Laboratory (ANL) is fundamentally an electrorefining technology which uses current flow to anodically oxidise uranium to form uranium ions in the molten salt electrolyte. At the cathode the uranium is reduced and electrodeposited as uranium metal.

The ANL process requires a metal feed. If oxide fuels are to be treated, it is necessary to reduce the uranium oxide (usually UO₂ pellets) to the metal. This reduction process is carried out chemically, using lithium metal in a LiCl or LiCl/KCl molten salt at 500 to 600°C. Alternatively, a salt transport process can be used involving a Cu-Mg-Ca alloy and molten CaCl₂ salt. However, in both reduction methods the by-products, Li₂O and CaO respectively, need to be recovered from the molten salt phase by an electrolysis step. Effectively this means a two stage process.

A disadvantage of the lithium reduction process for producing a metallic feed from an oxide is the production of Li₂O by-product. This requires recycle to make the process economic, and this is done by an electrolytic recovery of lithium metal. Hence this is a two stage process, comprising a reduction step followed by a lithium recovery stage.

More recently, in EP-A-1088113, there is proposed a method for the removal of oxygen from a metal oxide wherein an electrode comprising the metal oxide is contacted with a molten salt, and a potential is applied which is lower than the deposition potential of the cation of the molten salt, thereby facilitating removal of oxygen from the metal oxide.

Subsequently, in the PCT patent application published under No WO-A-01/41152, there is disclosed a single step process for reducing to metallic form a metal oxide present in spent nuclear fuel, the process comprising cathodically electrolysing the oxide in the presence of a molten salt electrolyte, the potential of the cathode being controlled so as to favour oxygen ionisation over deposition of the metal from the cations present in the molten salt.

The process thereby involves the use of a single electrochemical process to reduce the metal oxide fuel to a metallic form, with oxygen, carbon monoxide and carbon dioxide produced as the only by-products. The potential of the cathode is maintained and controlled so that only oxygen ionisation occurs and not the deposition of the cations (eg Ca ions) in the fused salt. Typically, the oxide comprises an actinide oxide, such as uranium oxide or irradiated uranium oxide.

This process was then developed and applied to the separation of metals from a mixture of metal oxides such as occurs in spent nuclear fuel, which is a frequent requirement in the nuclear power industry. Thus mixtures of uranium and plutonium oxides, together with the oxides of other actinide metals, may additionally be contaminated with oxides of other, chemically active, metals such as, for example, those associated with fission products. Co-pending patent application No PCT/GB02/02402 teaches a method for the treatment of irradiated fuel which allows for the separation of uranium, and metals more noble than uranium, from such mixtures as are found in spent nuclear fuel, and facilitates the provision of these metals in a form suitable for use as the feed in a molten salt electrorefining process, whilst ensuring that other, more electropositive, metals remain in the form of oxides.

The present inventors, however, recognised that there is frequently the requirement, both within the nuclear industry and the wider chemical industry, for the separation of metals from mixtures of metal oxides, and that the established technologies within these industries often provide inadequate means for the performance of such separations. Thus, whilst the prior art, as previously discussed, has focused largely on applications within the nuclear power industry and, most particularly, on processes involving actinide metals, it is often necessary, in a wide range of industries, to separate a large variety of metals, many of which are not members of the actinide series.

The present invention, therefore seeks to provide a method for the electrochemical separation of metals, the method relying on the different reduction potentials of different oxides which results in the reduction of one oxide to the free metal, whilst the other metal remains as the oxide. Examples of metals which might be separated in this way include transition metals, lanthanides and actinides.

### Statements of Invention

Thus, according to the present invention, there is provided a process for the separation of metals, said metals being comprised as the metal oxides in a mixed oxide sample, the process comprising:
(i) adding the mixed oxide to a molten salt electrolyte and cathodically electrolysing the oxide, the potential of the cathode being controlled so as to favour oxygen ionisation over deposition of metal from the cations present in the molten salt, and the applied potential difference being such as to facilitate selective reduction of one metal oxide at the expense of other metal oxides; and
(ii) separating the metal from the remaining metal oxides,
wherein the metal oxides wherein comprise oxides of metals from at least one of the transition metal, lanthanide or actinide series.

The potential of the cathode is maintained and controlled so that only oxygen ionisation occurs and not the deposition of the cations (eg Ca ions) in the fused salt, and also to ensure that, whilst reduction of one of the metals occurs smoothly, the other metals are not reduced and remain in the anode as oxides. The only by-products which are produced are oxygen, carbon monoxide and carbon dioxide gases.

The process may be applied to the separation of a wide variety of metals of the transition, lanthanide and actinide series which are comprised as the oxides in mixed oxide samples. The broad usefulness and versatility of the method is illustrated by its applicability to the separation of metals from mixtures of two or more metal oxides. Thus, it is possible to apply the method of the invention to the separation of metals of the transition, lanthanide and actinide series comprised as the oxides in mixed oxide samples comprising oxides of one, two or three of the said series. In other words, the method of the invention facilitates the separation of metals from mixed oxide samples which comprise any of the following combinations:
(a) transition metal oxides only;
(b) lanthanide oxides only;
(c) actinide oxides only;
(d) at least one transition metal oxide and at least one lanthanide oxide;
(e) at least one transition metal oxide and at least one actinide oxide;
(f) at least one lanthanide oxide and at least one actinide oxide; or
(g) at least one transition metal oxide and at least one lanthanide oxide and at least one actinide oxide.

A specific example of a preferred application of the process is in the separation of hafnium, present as the oxide, in samples of zirconium oxide. Zirconium metal is widely used in the nuclear power industry in zircalloy cladding. However, hafnium serves as a poison in nuclear reactors and it is vital, therefore, that it should be removed from the zirconium metal prior to the incorporation of this material in cladding. Its removal is facilitated by the process of the present invention, wherein a suitable potential difference is applied in order to facilitate the reduction of zirconium oxide to zirconium metal whilst leaving the hafnium oxide unchanged.

The mixed oxide may be in any physical form, and this is generally dependent on the particular application from which it has resulted. For example, it may be provided as solid pieces of irregular size and shape, but it may also comprise a powder, an amorphous mass, or a dense solid agglomerate. In any event, the material may be treated according to the method of the present invention by connection to an electrical circuit such that it serves as the cathode during electrolysis. Connection to the circuit may be effected by any of the standard means well known to those skilled in the art.

Preferably the mixed oxide is in contact with the cathode of an electrochemical cell. The cathode could be in the form of a mesh basket. The molten salt electrolyte may be any suitable molten salt or mixture of such salts, for instance chloride salts, preferably CaCl₂ and/or BaCl₂. The anode may be any suitable inert anode, such as carbon.

The separation step, whereby the metal is separated from the remaining metal oxides, may comprise any of a number of techniques well known to those skilled in the art. Thus, for example, simple dissolution and solvent extraction techniques may be applicable; alternatively, heating and slagging methods could be appropriate. As a further alternative, additional electrochemical means may be employed to effect the separation.

Optionally, reduction of the selected metal oxide may be carried out in one particular molten salt, whilst separation of that metal from the other metal oxide or oxides is effected in a different molten salt composition. Alternatively, the two processes may be performed in the same molten salt.

### Detailed description of the Invention

In order to carry out an embodiment of the present invention, an electrolytic cell is assembled which has a carbon anode and a mesh basket cathode. A mixed oxide sample is placed in the mesh basket. The electrolyte consists of a molten salt or a mixture of such salts comprising, for example, chloride salts such as CaCl₂ or BaCl₂. A voltage is applied between the cathode and the anode. At the cathode the reaction involves the diffusion of oxygen atoms to the surface of the solid, followed by ionisation according to the reaction:

O + 2e⁻ → O²⁻.

The oxide ions which are produced dissolve in the electrolyte and are transferred to the anode where they are re-oxidised to produce oxygen gas. Further by-products include carbon monoxide and carbon dioxide. The potential at the cathode may be controlled, via a third reference electrode, to ensure that the reaction occurring at the cathode is oxygen ionisation and not deposition of the cations in the fused salt, and that only a selected metal oxide is reduced. Electrolysis at elevated temperatures results in an increased rate of oxygen diffusion, thereby also encouraging ionisation rather than metal deposition.

After electrolysis the mixed oxide sample is left in the form of a metal/metal oxide solid mixture at the cathode, with one of the metals having been reduced to the metallic form, whilst the other metals remain in the form of their oxides. This metallic/metal oxide product is then subjected to a suitable separation treatment.

## Claims

1. A process for the separation of metals, said metals being comprised as the metal oxides in a mixed oxide sample, the process comprising:
(i) adding the mixed oxide to a molten salt electrolyte and cathodically electrolysing the oxide, the potential of the cathode being controlled so as to favour oxygen ionisation over deposition of metal from the cations present in the molten salt, and the applied potential difference being such as to facilitate selective reduction of one metal oxide at the expense of other metal oxides; and
(ii) separating the metal from the remaining metal oxides.
wherein said metal oxides comprise oxides of metals from at least one of the transition metal, lanthanide or actinide series.

2. A process as claimed in claim 1 wherein said mixed oxide sample comprises a mixture of two or more metal oxides.

3. A process as claimed in claim 1 or 2 wherein said metals comprise zirconium and hafnium and said mixed oxide sample comprises mixed zirconium and hafnium oxides.

4. A process as claimed in any one of claims 1 to 3 wherein the mixed oxide is provided as solid pieces of irregular size and shape, a powder, an amorphous mass, or a dense solid agglomerate.

5. A process as claimed in any preceding claim wherein the oxide is located in a mesh basket which forms the cathode.

6. A process as claimed in any preceding claim wherein the molten salt electrolyte comprises at least one chloride salt.

7. A process as claimed in claim 6 wherein the chloride salt is CaCl₂ or BaCl₂.

8. A process as claimed in any preceding claim wherein the anode is a carbon anode.

9. A process as claimed in any preceding claim wherein the step of separating the metal from the remaining metal oxides is carried out by the use of dissolution and solvent extraction techniques, heating and slagging methods or electrochemical means.

10. A process as claimed in any preceding claim wherein said reduction of the selected metal oxide is carried out in one molten salt whilst separation of the metal from the other metal oxide or oxides is effected in a different molten salt composition.

11. A process as claimed in any one of claims 1 to 9 wherein said reduction of the selected metal oxide and said separation of the metal from the other metal oxide or oxides is performed in the same molten salt.

## Revendications

1. Procédé de séparation de métaux, lesdits métaux étant constitués des oxydes métalliques dans un échantillon d'oxyde mixte, ledit procédé comprenant les étapes consistant à :
(i) ajouter l'oxyde mixte à un électrolyte à base de sel fondu et électrolyser l'oxyde à la cathode, le potentiel de la cathode étant maîtrisé de façon à favoriser l'ionisation d'oxygène par rapport au dépôt de métal à partir des cations présents dans le sel fondu, et la différence de potentiel appliquée étant telle qu'elle facilite la réduction sélective d'un oxyde de métal au détriment des autres oxydes de métaux ; et
(ii) séparer le métal des oxydes métalliques restants,
dans lequel lesdits oxydes métalliques comprennent des oxydes de métaux provenant d'au moins une des séries des métaux de transition, des lanthanides ou des actinides.

2. Procédé selon la revendication 1, dans lequel ledit échantillon d'oxyde mixte comprend un mélange de deux ou plus de deux oxydes métalliques.

3. Procédé selon la revendication 1 ou 2, dans lequel lesdits métaux comprennent du zirconium et de l'hafnium et ledit échantillon d'oxyde mixte comprend des oxydes mixtes de zirconium et d'hafnium.

4. Procédé selon l'une quelconque des revendications 1 à 3, dans lequel l'oxyde mixte est fourni sous la forme de morceaux solides de taille et de forme irrégulières, d'une poudre, d'une masse amorphe ou d'un agglomérat solide dense.

5. Procédé selon l'une quelconque des revendications précédentes, dans lequel l'oxyde est situé dans un panier à mailles qui forme la cathode.

6. Procédé selon l'une quelconque des revendications précédentes, dans lequel l'électrolyte à base de sel fondu comprend au moins un sel chlorure.

7. Procédé selon la revendication 6, dans lequel le sel chlorure est CaCl₂ ou BaCl₂.

8. Procédé selon l'une quelconque des revendications précédentes, dans lequel l'anode est une anode à base de carbone.

9. Procédé selon l'une quelconque des revendications précédentes, dans lequel on effectue l'étape de séparation du métal à partir des oxydes métalliques restants en utilisant des techniques de dissolution et d'extraction avec un solvant, des procédés de chauffage et de scorification ou des moyens électrochimiques.

10. Procédé selon l'une quelconque des revendications précédentes, dans lequel on effectue ladite réduction de l'oxyde métallique choisi dans un sel fondu tout en effectuant la séparation du métal à partir de l'autre oxyde métallique ou des autres oxydes métalliques dans une composition de sel fondu différent.

11. Procédé selon l'une quelconque des revendications 1 à 9, dans lequel on effectue ladite réduction de l'oxyde métallique choisi et ladite séparation du métal à partir de l'autre oxyde métallique ou des autres oxydes métalliques dans le même sel fondu.

## Patentansprüche

1. Verfahren zur Trennung von Metallen, wobei die genannten Metalle als Metalloxide in einer gemischten Oxid-Probe umfasst sind, wobei das Verfahren umfasst:
(i) Hinzufügen des gemischten Oxids zu einem geschmolzenen Salz-Elekrolyten und kathodisches Elekrolysieren des Oxids, wobei das Potenzial so geregelt ist, dass die Sauerstoff-Ionisierung gegenüber der Abscheidung von Metall aus den in dem geschmolzenen Salz vorliegenden Kationen bevorzugt ist, und die angelegte Potenzial-Differenz derart ist, dass sie die selektive Reduktion eines Metalloxids auf Kosten der anderen Metalloxide erleichtert; und
(ii) Abtrennen des Metalls von den verbleibenden Metalloxiden, wobei die genannten Metalloxide Oxide von wenigstens einem Metall der Übergangsmetalle, Lanthanide oder Actinide umfassen.

2. Verfahren wie in Anspruch 1 beansprucht, worin die genannte gemischte Oxid-Probe eine Mischung aus zwei oder mehreren Metalloxiden umfasst.

3. Verfahren wie in Anspruch 1 oder 2 beansprucht, worin die genannten Metalle Zirkonium und Hafnium umfassen und die genannte gemischte Oxid-Probe gemischte Zirkonium- und Hafnium-Oxide umfasst.

4. Verfahren wie in irgendeinem der Ansprüche 1 bis 3 beansprucht, worin das gemischte Oxid bereitgestellt wird als feste Stücke von ungleichmäßiger Größe und Form, ein Pulver, eine amorphe Masse oder ein dichtes festes Agglomerat.

5. Verfahren wie in irgendeinem vorangehenden Anspruch beansprucht, worin sich das Oxid in einem Netzkorb befindet, welcher die Kathode bildet.

6. Verfahren wie in irgendeinem vorangehenden Anspruch beansprucht, worin der geschmolzene Salz-Elektrolyt wenigstens ein Chlorid-Salz umfasst.

7. Verfahren wie in Anspruch 6 beansprucht, worin das Chlorid-Salz CaCl₂ oder BaCl₂ ist.

8. Verfahren wie in irgendeinem vorangehenden Anspruch beansprucht, worin die Anode eine Kohlenstoff-Anode ist.

9. Verfahren wie in irgendeinem vorangehenden Anspruch beansprucht, worin der Schritt der Abtrennung des Metalls von den verbleibenden Metalloxiden unter Verwendung von Aufschluss- und Lösemittel-Extraktionsverfahren, Erhitzungs- und Verschlackungsverfahren oder elektrochemischen Mitteln durchgeführt wird.

10. Verfahren wie in irgendeinem vorangehenden Anspruch beansprucht, worin die genannte Reduktion des ausgewählten Metalloxids in einem geschmolzenen Salz durchgeführt wird, wohingegen die Abtrennung des Metalls von dem anderen Metalloxid oder -oxiden in einer anderen geschmolzenen Salz-Zusammensetzung bewirkt wird.

11. Verfahren wie in einem der Ansprüche 1 bis 9 beansprucht, worin die genannte Reduktion des ausgewählten Metalloxids und die genannte Abtrennung des Metalls von dem anderen Metalloxid oder den - oxiden im gleichen geschmolzenen Salz durchgeführt wird.
